

## UNITED STATES PATENT OFFICE

CHARLES S. MCNOWN, OF BUNKER HILL, INDIANA

## LEATHER PRESERVATIVE AND PROCESS OF APPLYING SAME

No Drawing.

Application filed December 16, 1929. Serial No. 414,589.

This invention relates to toughening leather, or the like so that it will have increased wearing life.

The chief object of this invention is to increase the resistance of leather, or the like, so that it will have a greater length of life than a piece not treated with the invention.

One feature of the invention consists in the water proofing of the leather, or the like, simultaneously with increasing the resistance thereof.

Another feature of the invention consists in retaining the flexibility of the leather when treated with the solution.

Another feature of the invention consists in the variation in the amount of drier that may be employed whereby different kinds of leather may be treated to attain the same degree of toughness or wear resisting qualities or to treat leather of like kind so that different degrees of flexibility can be obtained therein such as the difference in flexibility between sole leather and upper leather for shoes.

Merely by way of illustration, for the proportions of the ingredients can be varied somewhat, the following formula is included. Gum copal 3 ounces, oleate aluminum 3 ounces, turpentine asphaltum 3 ounces, spirits of turpentine 1½ ounces, turpentine japan one ounce, asbestos powder ½ ounce, coloring matter or pigment, as desired and required if a colored preservative is to be employed. Each of the ingredients above mentioned is a commercial product sold in the trade under the name herein used. Turpentine asphaltum is believed to be ground asphaltum cut with turpentine and is commonly used in lithographer's inks. Turpentine japan is a common drier for inks and paints and is believed to be japan gum dissolved in turpentine.

The gum copal is first dissolved in denatured alcohol or aniline oil. The oleate aluminum is dissolved in petroleum oil. The other ingredients are then added to the mixture of the two solutions. The asbestos powder consists chiefly of a very finely divided asbestos and might be termed an asbestos flour product although the size of the particles is

smaller than ordinary flour particles. The aniline oil is the product of that name used in the dyeing of certain silks, poplin, etc. and is believed to be aniline dissolved in poppy seed oil, china wood oil or a similar vegetable oil.

The ultimate mixture is a solution which preferably is applied to the flesh side of the leather although it can be applied to either or both sides. The leather before the application of the solution thereto must be dry. Preferably sole leather is roughened before the solution is applied thereto. This is to facilitate the quicker penetration of the solution into the pores of the leather.

The addition of the solution to the leather seems to fill the pores of the leather and serves to bind the fibers thereof together making the leather more resistant to wear and incidentally water proof but the solution before mentioned does not make brittle the leather in the toughening thereof. In other words the leather can be treated so that it is more firm and pliable than it was previous to the application of the solution.

For treating belting and sole leather the solution is applied to it until the leather is completely saturated therewith. Upper leather is not subjected to this extension treatment and likewise the solution may be modified so that the amount of gum copal is negligible therein or an intermediate amount may be employed if desired and when required.

The invention therefore consists in, first, the preparation of the solution per se, second, the constituents thereof in the proportions approximately indicated except when modified as hereinbefore noted and third, the application of the same to leather or like material.

While the invention has been described in great detail and with considerable exactness in the foregoing specification the same is in no sense to be considered as restrictive in character but the various modifications of this invention which will readily suggest themselves to those skilled in the art to which the same applies are all to be understood to be within the broad purview of the invention,

reference being had to the appended claims.

The invention claimed is:

1. A solution suitable for treating leather, and the like to increase its wearing qualities
- 5 comprising a solution including gum copal, oleate aluminum, turpentine asphaltum, spirits of turpentine, turpentine japan and asbestine powder.
- 10 2. A solution suitable for treating leather, and the like to increase its wearing qualities comprising a solution including gum copal, oleate aluminum, turpentine asphaltum, spirits of turpentine, turpentine japan, asbes- tine powder and coloring matter.
- 15 3. A solution suitable for treating leather, and the like to increase its wearing qualities comprising a solution including the follow- ing ingredients in approximately the propor- tions enumerated, gum copal three ounces,
- 20 oleate aluminum three ounces, turpentine asphaltum three ounces, spirits of turpentine one and one-half ounces, turpentine japan one ounce, asbestine powder one-half ounce, color- ing matter or pigment, as desired and re- quired.
- 25 4. A solution suitable for treating leather,

and the like to increase its wearing qualities comprising a solution including gum copal, oleate aluminum, asbestine powder, and tur- pentine.

5. The process of preparing a solution suitable for treating leather, and the like to increase its wearing qualities comprising forming a solution of gum copal in denatured alcohol, forming another solution of oleate aluminum in petroleum oil, and then mixing the same together and with turpentine asphaltum, spirits of turpentine, turpentine japan and asbestine powder.

6. The process of preparing a solution suitable for treating leather, and the like to increase its wearing qualities comprising forming a solution of gum copal in aniline oil, forming another solution of oleate alum- inum in petroleum oil, and then mixing the same together and with turpentine asphaltum, spirits of turpentine, turpentine japan and asbestine powder.

In witness whereof, I have hereunto affixed my signature.

CHARLES S. McNOWN.

90

80

95

85

100

49

105

45

110

50

115

55

120

60

125

61

130